

# UNITED STATES PATENT OFFICE.

FRANCIS C. FRARY, OF MINNEAPOLIS, AND STERLING N. TEMPLE, OF ST. PAUL, MINNESOTA; SAID TEMPLE ASSIGNOR OF ONE-SIXTH OF THE WHOLE RIGHT TO SAID FRARY.

## LEAD ALLOYS CONTAINING A PLURALITY OF THE METALS OF THE ALKALINE EARTHS.

1,158,672.

Specification of Letters Patent.

Patented Nov. 2, 1915.

No Drawing.

Application filed July 31, 1915. Serial No. 43,010.

*To all whom it may concern:*

Be it known that we, FRANCIS C. FRARY and STERLING N. TEMPLE, citizens of the United States, residing at Minneapolis and

5 St. Paul, respectively, in the counties of Hennepin and Ramsey, respectively, and State of Minnesota, have invented certain new and useful Improvements in Lead Alloys Containing a Plurality of the Metals 10 of the Alkaline Earths; and we do hereby declare the following to be a full, clear, and exact description of the invention, such as will enable others skilled in the art to which it appertains to make and use the same.

15 Our invention has for its object to provide an improved metallic alloy having certain characteristics especially adapting it for use in the casting of type and similar articles in molds, and in the manufacture of bullets 20 and other forms of ammunition.

In the manufacture of type metal, hardness and resistance to compression without cracking are necessary, and furthermore, the metal employed must be of such character 25 that it will not contract on solidifying, but, on the contrary, will slightly expand and fill the mold in which it is cast. In the manufacture of ammunition, it is very desirable that the alloy be hard and that its 30 specific gravity be as high as possible, so as to thereby concentrate the maximum of kinetic energy in a minimum volume.

Certain of the above noted desirable characteristics have hitherto been produced by 35 adding a considerable proportion of antimony to lead. The antimony, however, reduces appreciably the specific gravity of the alloy. Furthermore, antimony, especially at the present time, is very expensive, as compared with lead, and because of the considerable amount thereof necessarily employed, 40 makes the alloy expensive.

In carrying out our invention, we use small quantities of a plurality of the metals 45 of the alkaline earths (magnesium, calcium, strontium and barium) in a main body of lead.

We are aware that many persons do not consider magnesium as a metal of the alkaline earths. However, in its properties, it 50 more closely resembles calcium, barium and strontium than it does the other members of the second group of the "periodic system,"

and we believe it to be properly classed with calcium, barium and strontium, and, hence, 55 have so considered it in this application.

Experiments which we have made have demonstrated that by an expenditure of a given amount of money for the metals to be added to the lead, a much harder and 60 heavier alloy can be produced by the use of a plurality of the above noted metals of the alkaline earths, than can be obtained by the use of any one thereof, alone, with the lead. 65

We have also found that by the use of less than two per cent. in all of such a plurality of the metals of the alkaline earths, the alloy may be made as hard as commercial antimonial lead, or harder than the same. We 70 have further found that the alloy containing a plurality of the metals of the alkaline earths may be improved and made still harder by the addition of a small amount of copper. This addition also makes the 75 alloy tougher, and prevents it from having the brittleness which characterizes ordinary antimonial lead.

As examples of hard lead alloys made in accordance with our invention, the following formulae are given: 1. 98.75 parts lead, 0.5 parts calcium and 0.75 parts barium. 2. 98.7 parts lead, 0.5 parts calcium, 0.6 parts barium and 0.2 parts copper. 3. 98.89 parts lead, 0.37 parts calcium, 0.33 parts barium, 80 0.24 parts strontium, and 0.17 parts copper. 4. 98.69 parts lead, 0.34 parts calcium, 0.43 parts barium, 0.19 parts strontium, 0.1 parts magnesium and 0.25 parts copper. 5. 98.7 parts lead, 0.42 parts calcium, 0.56 parts 85 barium, 0.12 parts magnesium, 0.2 parts copper. 6. 98.76 parts lead, 0.41 parts calcium, 0.46 parts strontium, and 0.37 parts copper. 7. 99.35 parts lead, 0.5 parts calcium, and 0.15 parts magnesium. 95

Comparing the above given examples of the different alloys made in accordance with our invention, all but examples 6 and 7 are decidedly harder than the hardest commercial antimonial lead. Examples 6 and 7 are 100 nearly as hard as this antimonial lead. Example 4 is the hardest of all of those given, while examples 1, 2, 3 and 5 are a little softer than example 4, but distinctly harder than antimonial lead. 105

Commercial lead, as well as pure lead, is

in this specification and in the claims intended to be included and covered by the term "lead." It is a well known fact that commercial lead contains small quantities 5 of copper and some other materials not removed in the process of purification. Frequently commercial lead will contain as large an amount of copper as would be desired in the alloy, and in this case a further 10 addition of copper would not, of course, be needed.

What we claim is:

1. As a new article of manufacture, a metallic alloy containing lead and a plurality of the metals of the alkaline earths. 15
2. As a new article of manufacture, a metallic alloy containing lead, a plurality of metals of the alkaline earths, and copper. 20
3. As a new article of manufacture, a hard lead alloy consisting of a main body of lead, to which has been added a small amount of a plurality of the metals of the alkaline earths. 25
4. As a new article of manufacture, a hard lead alloy, consisting of a main body of lead, to which has been added a small quantity of a plurality of the metals of the alkaline earths, and a small amount of copper. 30
5. As a new article of manufacture, a hard lead alloy consisting of a main body of lead, and a plurality of the metals of the alkaline earths in an amount less than two per cent. 35

6. As a new article of manufacture, a 35 tough hard lead alloy, consisting of a main body of lead, a plurality of the metals of the alkaline earths in an amount less than two per cent., and a small amount of copper.

7. As a new article of manufacture, a 40 hard lead alloy consisting of a main body of lead to which have been added small quantities of at least three of the metals of the alkaline earths, (magnesium, calcium, strontium, and barium.) 45

8. As a new article of manufacture, a hard lead alloy consisting of a main body of lead to which have been added small quantities of at least three of the metals of the alkaline earths, (magnesium, calcium, strontium, and barium,) 50 and also a small amount of copper.

9. As a new article of manufacture, a hard lead alloy consisting of a main body of lead and small amounts of magnesium, 55 calcium, strontium, and barium.

10. As a new article of manufacture, a hard lead alloy consisting of a main body of lead and small amounts of magnesium, calcium, strontium, and barium, and also a 60 small amount of copper.

In testimony whereof we affix our signatures in presence of two witnesses.

FRANCIS C. FRARY.  
STERLING N. TEMPLE.

Witnesses:

CLARA DEMAREST,  
F. D. MERCHANT.